

Oct. 27, 1925.

1,559,335

B. S. McCONNELL

METHOD OF FILLING THE INTERSTICES BETWEEN THE UNITS OF A PAVEMENT OR FLOOR

Filed Oct. 4, 1921

Fig. 1.



Fig. 2.



Inventor:  
Bertram S. McConnell,

by Dodge and Dow  
Attorneys

## UNITED STATES PATENT OFFICE.

BERTRAM S. McCONNELL, OF INDIANAPOLIS, INDIANA, ASSIGNOR TO PETER C. REILLY, OF INDIANAPOLIS, INDIANA.

METHOD OF FILLING THE INTERSTICES BETWEEN THE UNITS OF A PAVEMENT OR FLOOR.

Application filed October 4, 1921. Serial No. 505,284.

To all whom it may concern:

Be it known that I, BERTRAM S. McCONNELL, a citizen of the United States, residing at Indianapolis, in the county of Marion and State of Indiana, have invented certain new and useful Methods of Filling the Interstices Between the Units of a Pavement or Floor, of which the following is a specification.

- 10 This invention relates to a method of filling the interstices between the units of a pavement or floor composed either of brick, asphalt, or wooden blocks, the method being such as to produce a solidified filler as well  
 15 as to form a bond between the component elements of the pavement or floor. The materials employed are such that they may be readily placed in the joints and thereafter so treated as to produce a substantially co-  
 20 herent mass which also adheres to the contiguous faces of the blocks, thereby forming a perfect bond between the various elements, thus producing in effect a continuous surface. Various methods and materials are at  
 25 present employed in filling the spaces or interstices, but such methods are more or less wasteful and are not effective as a filler and a bond.

Due to the narrow interstices or narrow openings it is oftentimes difficult, in the present methods, to thoroughly fill such openings or interstices. Where liquid bituminous material is employed it is often found that an inadequate amount of such material is present in the interstices and frequently the material will congeal upon the upper marginal portions of the blocks and only a small amount will enter between them. Thus there is produced an inadequate filling and there is likewise present upon the exposed pavement surface material which is harmful to the surface besides being wasteful. Again, if the units are spaced apart to any considerable degree, such material runs down through the interstices and under the units, distorting the surface of the pavement or floor, frequently leaving the interstices unfilled. These objections are present not only with hot bituminous liquid but also with a cold bituminous liquid. When sand, cement, sawdust

or other granular material are used, separately or in mixture, they possess but little adhesive qualities to bond the various blocks together and they are apt to work down under the blocks, thereby causing the surface to become uneven.

Two embodiments of the present invention are shown in the annexed drawings where-  
 in:

Figure 1 is a sectional elevation of a portion of a pavement, disclosing wooden blocks having the interstices between the same filled or closed with the material as herein-  
 after set forth; and

Figure 2, a perspective view showing a similar pavement wherein the body of the pavement is formed by bricks or asphaltic blocks.

With the present invention I propose to use asphalt, coal tar, coal tar pitch, petroleum pitch, and other like substances which may be reduced by distillation to a point where the material becomes dry, and, to a certain extent, brittle, without losing its inherent plasticity and adhesive properties. In this condition such materials can be reduced to powdered form by crushing or granulating and such form will be retained until exposed to an excessive heat or to the action of some suitable solvent. The material thus powdered may be swept into the interstices until all the interstices are completely filled with it, the material being swept clean from the surface of the pavement or floor. In one form of the invention the floor is then subjected to a dressing, either by a spray or brush, of a solvent, such as solvent naphtha, naphthalene, phenanthrene, creosote oil, or any other suitable substance, either hot or cold, as required, according to the nature of the solvent employed. Such solvent material transforms the granular or powdered mass into a homogeneous body and thoroughly seals and fills the interstices. At the same time, owing to the coherent nature of the material employed, a bond is formed thereby with the adjacent faces of the blocks.

In Figure 1, I have shown a series of wooden blocks denoted by 1 and the filling material denoted by 2. In Figure 2, the

body which may be made of asphaltic blocks or bricks is denoted by 3, while the plastic filling material is denoted by 4.

Another manner of producing this bond 5 is as follows:

One may take, say four parts of powdered plastic base material, such as bitumen, and mix the same thoroughly with one part 10 granular solvent, by turning the two over together at least three or four times, or running the same through a concrete mixer. Such granular solvent may take the form of sawdust soaked in a material which has a 15 solving action upon the plastic base. The material thus intermixed, namely the base and the granular solvent or the carrier impregnated with the solvent, is then worked into the interstices until they are entirely filled, which may be readily done with a 20 broom or a squeegee. It is essential that the mixture be swept immediately into place before any fusing action obtains between the filler and the solvent. The surface of the pavement is then preferably flushed 25 with creosote oil which is to be quickly forced into the interstices by a rubber squeegee. Such material will be absorbed by the filler and the squeegee will clean 30 off the surface entirely. If the openings or 35 interstices are large it may be necessary to repeat the operation after the filler has settled. The filler, however, is of such a nature that the operation above set forth can be easily repeated until all the voids are entirely filled. Complete fusing of the filler 40 obtains within about twenty-four hours.

Again, instead of using a liquid solvent or the carrier for the solvent, as just specified, powdered bitumen may be mixed with 45 powdered or crystal naphthalene or phenanthrene, or other granular solvent, prior to its being swept into the interstices, after which it will be subjected to the application of heat, as by the use of a blow torch or a 50 jet of live steam, which will serve to soften the powdered plastic and cause it to pass into a cohesive and bonding relation with the blocks, at the same time filling in the interstices or openings, where it will remain.

The invention is susceptible of wide application and has been found highly efficient and effective in actual use.

The use of these high point boiling materials renders the filling and the bond produced thereby, immune to the action of ordinary atmospheric temperatures. That is to say, the material will not soften to such an extent as to flow even when subjected to 60 the direct action of the sun rays.

What is claimed is,—

1. That method of filling the joints between contiguous paving or flooring elements, which consists in supplying said 65 joints with a hydrocarbon material normal-

ly non-fluent under atmospheric temperatures, and temporarily softening the same when in situ to cause such material to coalesce and to bond the contiguous faces of the elements aforesaid.

2. That method of filling the joints between contiguous paving or flooring elements, which consists in supplying said joints with a comminuted hydrocarbon material normally non-fluent under atmospheric temperatures, and temporarily softening the same when in situ to cause such material to coalesce and to bond the contiguous faces of the elements aforesaid. 70 75

3. That method of filling the joints between contiguous paving or flooring elements, which consists in supplying said joints with a hydrocarbon material normally non-fluent under atmospheric temperatures, and temporarily softening the same 80 when in situ by a solvent agent whereby the material is caused to coalesce and to bond the contiguous faces of the elements aforesaid. 85

4. That method of filling the joints between contiguous paving or flooring elements which consists in supplying said joints with a normally hard material produced from hydrocarbon, said material being normally non-fluent at atmospheric temperatures, and thereafter temporarily softening the same when in situ whereby the material is caused to coalesce and to form a bond with the contiguous faces of the elements aforesaid. 90 95

5. That method of filling the joints between contiguous paving or flooring elements which consists in supplying such joints with a mass containing a normally non-fluent material produced from a hydrocarbon, and thereafter temporarily softening the same when in situ whereby the elements are bonded and the mass becomes substantially solid throughout. 100 105

6. That method of filling the joints between contiguous paving or flooring elements, which consists in supplying such joints with a mass of powdered hydrocarbon of high boiling point, and thereafter causing said powder to coalesce into a substantially solid body. 110 115

7. That method of filling the joints between contiguous paving or flooring elements, which consists in supplying said joints with a normally hard material produced from hydrocarbon, said material being normally non-fluent at atmospheric temperatures, and introducing into the joints with such material a carrier soaked with a solvating substance for such material. 120 125

8. That method of filling the joints between contiguous paving or flooring elements, which consists in supplying said joints with a normally hard material produced from hydrocarbon, said material be- 130

ing normally non-fluent at atmospheric temperatures, and likewise introducing into said joints a body of sawdust saturated with a solvent for such hydrocarbon material.

5. 9. That method of filling the joints between contiguous paving or flooring elements, which consists in supplying said joints with a normally hard material produced from hydrocarbon, said material be-

ing non-fluent at atmospheric temperatures, and likewise introducing into the joints a body of sawdust saturated with a solvent for such hydrocarbon material, and finally flushing the joints thus filled with creosote oil.

In testimony whereof I have signed my name to this specification.

BERTRAM S. McCONNELL.